

## UNITED STATES PATENT OFFICE

IRVING F. LAUCKS AND GLENN DAVIDSON, OF SEATTLE, WASHINGTON, ASSIGNEES TO  
I. F. LAUCKS, INCORPORATED, OF SEATTLE, WASHINGTON, A CORPORATION OF  
WASHINGTON

## GLUE AND METHOD OF MAKING

No Drawing. Original application filed October 29, 1923, Serial No. 671,381. Divided and this application  
filed October 4, 1928. Serial No. 310,431

The art of making a water-proof glue from certain protein materials has been known for some time; thus casein and blood albumin are in common use. These last mentioned 5 compounds, however, have a number of disadvantages from a practical standpoint. Casein is costly and lack of uniformity in the material as derived from various sources is a serious detriment; while blood albumin 10 is not available except in certain situations. There is accordingly a great demand, particularly in the veneer industry where large quantities of glue are consumed, for a new glue that will be cheap and at the same time 15 sufficiently water-proof.

By water-proof, in this connection, it is not meant that glues thus characterized will resist the action of water indefinitely, but it is meant that they are water-proof in the 20 sense in which the term is used in the veneer industry, viz., that a panel can be soaked in cold water for from seventy-two to one hundred hours, or in boiling water for eight hours, without separation.

25 Vegetable compounds have not, so far as we are aware, been heretofore satisfactorily employed as a basis for water-proof glues of the type in question. It is true that some veneer makers, on account of the high price 30 of casein, have come to use starch glues but these, at least as heretofore made, are not at all water-proof, and vegetable proteins have not heretofore been used at all, so far as we are aware.

35 We have now discovered, however, that by subjecting the same to proper treatment, vegetable matter containing proteins in proper amount, can be converted into a water-proof glue that will satisfy the rigid requirements of veneer making. The requisite raw 40 material may be derived from a number of sources and the treatment of such material is relatively simple and inexpensive so that as a result we are able to produce a satisfactory 45 glue at a much lower cost than has heretofore been possible.

To the accomplishment of the foregoing and related ends, the invention, then, consists of the combination of ingredients or composition of matter and the steps involved in the

preparation of such composition hereinafter fully described and particularly pointed out in the claims, it being understood that such disclosed ingredients and steps constitute but several of the various ways in which the 55 principle of the invention may be used.

We have found that soya bean flour constitutes an admirable raw material for our purpose. Such flour is preferably made by grinding soya bean cake so that 80 per cent. 60 will pass a 100 mesh screen and when treated with certain chemicals, or other substances, we make therefrom a very satisfactory glue that meets the requirements of the veneer trade fully and is in many respects better 65 than the usual glues now on the market. Such bean cake, as analyzed by us, is found to contain on the average 45 per cent. protein, 12 per cent. water, 5 per cent. cellulose, 70 or crude fibre, 7 per cent. oil, 6 per cent. ash, and 25 per cent. carbohydrates.

We do not, however, wish to limit ourselves to soya bean flour or to vegetable protein derived from this source.

Soya bean flour made from soya bean cake 75 from which the oil has been expressed, is preferably used in practice because it is cheaper and makes a better glue, but flour made from whole soya beans, without expressing the contained oil, may also be used, 80 although obviously this would not be economical in view of the value which attaches to such oil. As to the fineness of the flour, it is not necessary that the meal be ground as fine 85 as indicated above, but fineness is desirable from a practical standpoint.

When the usual chemicals employed in making casein glue, viz., lime and sodium silicate, are added to a vegetable protein-containing material, for example, soya bean flour, a glue results, but it is not as good as casein glue. It is not as highly water resistant nor as workable. We find, however by the use of caustic soda with such vegetable 95 protein-containing matter, a much better glue is obtained, such caustic soda apparently playing the part of dispersing the colloidal material. The resultant glue is then somewhat similar in its working properties to 100

casein glue, although its water resistance is still slightly less.

Preferably we react on our vegetable protein-containing material with both caustic soda and lime. As equivalents of such caustic soda, caustic potash and ammonia may be used, although more expensive. Other equivalents of caustic soda are salts of soda (or potash) with weak acids, e. g. sodium phosphate, sodium borate and the like, when lime is present. Similarly in place of lime, magnesia, baryta and strontia may be used as equivalents.

In order to improve the working properties, e. g. the spreading and flow, of the glue produced as aforesaid as well as the water resisting properties, we have found it desirable to add other substances of which the following are examples:

20 Carbon bisulfide, calcium polysulfide. Equivalents would be other sulfur compounds of like properties or constitution.

Copper sulfate, cuprammonium compounds, copper-caustic soda compounds.

25 Equivalents would be other alkaline compounds of copper.

Sodium dichromate. Equivalents would be other metallic dichromates or chromates.

30 Chrome alum, ammonia alum, aluminum sulfate. Equivalents would be other alums and aluminum salts, including aluminates.

Quebracho, sumach, spruce extract (concentrated sulfite liquor). These are all commonly used tanning agents. Equivalents 35 would be other vegetable tanning agents.

Zinc sulfate, zinc chloride, ammonium zincate. Equivalents would be other zinc compounds.

40 Calcium sulfate, calcium oxychloride (bleaching powder). Equivalents would be other calcium salts, or alkaline earth salts.

Cresylic acid. Equivalents would be other phenols.

45 Rosin, sodium or calcium soaps of rosin. Equivalents would be other resins or resin combinations with metals.

50 Carbon bisulfide imparts very great water resisting properties, as does also calcium polysulfide, although to a lesser degree; the copper salts and the dichromates make the glue more readily workable while at the same time imparting increased water resistance; the alums, the tanning agents, zinc compounds, calcium compounds and cresylic acid 55 increase the water resistance of the glue; the silicates and related compounds act as thinners while at the same time increasing the water resistance and the strength of the glue; and the rosin and derivatives thereof act as

60 thinners and make the glue more readily workable. Substances such as the foregoing, which act as a thinner, or render the glue more readily workable, may be appropriately referred to as spreaders.

65 It has also been found desirable to add to

the basic glue composition produced by reacting on protein containing vegetable matter, as described above, other substances which act as retarders, e. g. calcium chloride and sodium chloride. A retarder, in this connection, it should be explained, is a substance which prevents the wet glue after mixing from setting to a jelly or otherwise thickening so that it can not be spread. This action, however, is only important in the case of a few of the formulæ that we have used and most of our glue mixtures have not required the addition of such a retarder.

We have also found that certain substances, in conjunction with lime, will act in the same way as the caustic soda and also as thinners, e. g. sodium phosphate, sodium perborate and sodium sulfite. These salts are all related in that they are combinations of the strong base sodium with a weak acid and there are a number of other salts that fall in the same category and which have a similar effect, so need not be listed in detail.

As examples we may cite the following typical formulæ:

(1) Mix 30 parts soya bean flour with 120 parts water; add 13 parts of 18 per cent. caustic soda solution and mix; 5 parts carbon bisulfide are then added and stirred well; to this 3 parts calcium hydrate are added and stirred in; then 15 parts water glass (sodium silicate) are stirred in; finally, add 1 part copper sulfate to 5 parts of water and stir in. This makes the finished glue, which is then spread on panels, for example, put under pressure for several hours, whereupon the pressure may be released.

(2) Mix 15 parts soya bean flour with 1 part sodium dichromate; add 40 parts water and 13 parts 18 per cent. caustic soda solution; stir well; then add 2 parts calcium hydrate in 30 parts of water, giving finished glue.

(3) Mix 30 parts soya bean flour, 5 parts rosin, 1½ parts copper sulfate, 1 part quebracho together dry; add 90 parts water and 26 parts 18 per cent. caustic soda solution; stir well; add 6 parts calcium hydrate in 15 parts water; then add 15 parts water glass, giving finished glue.

(4) Mix dry, 40 parts soya bean flour, 6 parts rosin, 8 parts Portland cement, 3 parts dichromate of soda and 5 parts caustic soda; add 140 parts water and 14 parts water glass; stir well; add 50 parts water.

(5) Mix 30 parts soya bean flour, 1 part alum, 70 parts water; add 13 parts 18 per cent. caustic soda solution and 4 parts calcium hydrate in 20 parts water.

(6) Mix 30 parts soya bean flour, 1 part sodium dichromate, 0.1 part zinc sulfate, 80 parts water; add 13 parts 18 per cent. caustic soda solution and 4 parts calcium hydrate in 20 parts water.

(7) Mix 30 parts soya bean flour, 5 parts rosin,  $1\frac{1}{2}$  parts copper sulfate,  $\frac{1}{2}$  part sodium dichromate, 90 parts water, 1 part creyslic acid, 26 parts 18 per cent. caustic soda solution, 6 parts calcium hydrate in 15 parts water, 15 parts water glass.

20 parts of lime, and subsequently incorporating a caustic soda solution to spreading consistency.

IRVING F. LAUCKS.  
GLENN DAVIDSON. 70

The particular order in which the several ingredients are admixed together in the formulæ just given may be varied, and it is not necessary that the manufacture of the product be completed in a single continuous operation, but as a matter of practice we have found it desirable in certain cases to mix only certain of the ingredients initially and then add the others just before the glue is required for use. Thus, the glue that we are at present making commercially is made as follows, viz:—soya bean flour, lime, rosin and potassium dichromate are mixed dry, and in this form is shipped to the veneer plants. In the latter such dry product is then mixed with water, caustic soda solution and sodium silicate in the form of water glass, thereby making the finished glue. The proportions in which the foregoing ingredients are employed in the case of the particular method of manufacture just described will be substantially as given in the preceding formulæ numbered (1) to (7), inclusive.

30 It will also be understood, of course, that the foregoing formulæ are typical and that many variations are actually made therein in the compounding of our improved glue.

This application is a division of our application Serial No. 671,381, filed October 29, 1923 (now Patent No. 1,689,732).

Other modes of applying the principle of our invention may be employed instead of the one explained, change being made as regards the process herein disclosed or the materials employed in carrying out such process provided the stated ingredients and steps or the equivalent of such stated ingredients or steps be employed.

45 We therefore particularly point out and distinctly claim as our invention:—

1. The process of making an adhesive, which comprises dry mixing soya bean flour with an alkaline earth hydroxide, and subsequently incorporating an alkali metal hydroxide and water.

50 2. A process of making an adhesive, which comprises dry-mixing soya bean flour with a compound of an alkali-forming metal, and subsequently incorporating an alkaline medium and water to spreading consistency.

3. The process of making an adhesive, which comprises dry mixing soya bean flour with lime, and subsequently incorporating a caustic soda solution.

55 4. The process of making an adhesive, which comprises dry mixing soya bean flour with lime, in the proportion of about 100 parts of the soya bean flour and about 10 to

75

80

85

90

95

100

105

110

115

120

125

130